

Sept. 23, 1952

R. B. KELLER ET AL

2,611,313

DUPLICATING METHOD

Filed Dec. 10, 1946

FIG.1.



FIG.2.



FIG.3.



FIG.4.



FIG.5.



FIG.6.

INVENTORS.

RAY B. KELLER  
BY HARROLD B. DAWSON

J. C. Miseney  
ATTORNEY.

## UNITED STATES PATENT OFFICE

2,611,313

## DUPLICATING METHOD

Ray Bennett Keller and Harold Bowman Dawson, Erie, Pa., assignors to Hammermill Paper Company, Erie, Pa., a corporation of Pennsylvania

Application December 10, 1946, Serial No. 715,308

2 Claims. (Cl. 101—149.4)

1

The present invention relates to the duplicating art and more particularly, provides a novel method for duplicating which method is of the type generally referred to as spirit duplicating. The present invention also provides a novel master sheet for use in spirit duplicating and a manifold assembly including such master sheet.

In the known processes of spirit duplicating, special duplicating inks or duplicating carbon paper is used to form a master copy of drawings, or matter written by hand or by typewriter. Such master copy is formed on a blank sheet of especially suitable paper or other material referred to as the master sheet, the ink or carbon being applied to the master, only along the desired lines to be duplicated, either by hand or by transfer from the carbon sheet. The duplicating ink or carbon is soluble in a duplicating fluid such as alcohol, water or other suitable solvent with which the copy sheets or the master sheet is moistened for the production of multiple copies. In most instances the duplicating fluid comprises an alcohol mixture and thus the definition "spirit duplicating" has been adopted.

Since copies are made directly from the master sheet, the data thereon must be in the form of a mirror image. The present invention is adapted for use in the direct process.

One of the most frequently used systems for forming a master sheet will be described in order that the later description of the present invention may be fully understood. For the preparation of a direct process master sheet according to this known process a sheet of "duplicating carbon" is placed in a typewriter with the coated side facing outwardly. The master sheet is superimposed upon the coated surface of the duplicating carbon. When the typewriter is operated, the type bars will strike the outer surface of the master sheet and the pressure or impact thereof will cause the transfer of duplicating material from the duplicating carbon to the back surface of the master sheet. Obviously, the letters thus formed on the back surface of the master sheet will be mirror images and will be formed of the duplicating material. The copy sheets may be moistened with the solvent and brought into contact with the master sheet. Alternatively the master sheet thus formed may itself be moistened a number of times with the proper solvent and placed in contact with the desired number of copy sheets. In either event a portion of the duplicating material in the mirror images on the master sheet will be transferred to each of the successively presented copy sheets.

2

The nature of the duplicating ink or carbon is such as to be extremely likely to smudge or stain the fingers of the operator and soil or mar the surface of the master sheet with the result that imperfect reproductions are formed. Various proposals have been made for applying a protective coating over the coating of duplicating material on the duplicating carbon sheet to prevent such smudging. However such proposals offer only a protective film and do not embody the new duplicating process herein disclosed. Furthermore it will be apparent that when portions of the coatings on the duplicating sheet are transferred to the master sheet, as in the typewriting operation described above, the protective coating will first be brought into contact with the master sheet. The volume of duplicating material available in each letter or figure for the production of copies is reduced at least to the extent that a part of the material transferred to the master sheet is not a duplicating material.

The present invention provides an entirely different form of master sheet which is itself coated continuously on one face thereof with a suitable duplicating material. A protective coating of non-duplicating material is placed over the first-mentioned coating. The protective coating is preferably insoluble in the solvent to be used and is such as to be much more adherent to a backing sheet of paper or the like, when struck by a type bar, than it is to the duplicating material on the master sheet. Thus, in the use of the present invention, a backing sheet is placed next to the platen of the typewriter and the master sheet is placed thereover with the protective coating against the backing sheet. When the typewriter is operated, impact or pressure of the type bars will transfer the material of the protective coating to the backing sheet. When the backing sheet and master sheet are separated, the duplicating material within the area of the letters or figures on the type bars will be exposed. It will be apparent that the prepared master sheet will have an almost continuous coating of protective material thereon which coating is broken only in the localized areas where mirror images of the letters or figures appear. The master sheet may be brought into contact with moistened copy sheets for the production of copies or, if so desired, the master sheet may itself be moistened whereby to produce copies on dry sheets of copy paper.

Certain preferred forms and illustrative manners of use of the present invention will be specifically described hereinbelow. Such specific

descriptions taken in connection with the drawings accompanying and forming a part of this specification will enable those skilled in the art to make use of the present invention in various forms and manners.

In the drawings:

Fig. 1 is a fragmentary sectional view of a master sheet embodying one form of the present invention;

Fig. 2 is a view similar to Fig. 1 but showing a modified form;

Fig. 3 is a diagrammatic view showing the master sheet of Fig. 2 and a backing sheet in assembled position on the platen of a typewriter;

Fig. 4 is a fragmentary sectional view illustrating in exaggerated diagrammatic form a portion of the master sheet shown in Fig. 2 after impact by the type bars of a typewriting machine;

Fig. 5 is a view similar to Fig. 4 showing the prepared master sheet and the backing sheet 20 after separation; and

Fig. 6 is a fragmentary sectional view of a modified form of the present invention in which the master sheet is shown assembled as in a salesman's order book and the like.

Referring first to Fig. 1, the master sheet of the present invention comprises a base sheet 1 of paper, regenerated cellulose, metal foil, glassine, or other flexible sheet material normally used in the manufacture of master sheets. The base sheet 1 has formed thereon a layer or a coating 2 of any suitable duplicating material. The duplicating material may be of the type ordinarily used in the manufacture of duplicating carbon sheets obtainable in the market. Such material may be made from a suitable combination of various waxes, oils and dyestuffs and be of such nature that it is sufficiently soluble in a duplicating fluid such as an alcohol mixture or other solvent that upon repeatedly moistening the same with the solvent, a portion thereof may be repeatedly transferred to copy sheets in the manner familiar in the art.

In accordance with the present invention, a continuous coating 4, which will be identified herein as a protective layer, is laid upon the exposed surface of the layer 2 of duplicating material. The protective layer is made of a material which has a sufficient affinity for the layer 2 of duplicating material that it will remain united therewith except where it is dislodged as described below. The protective material must have the general characteristics of the waxy compositions normally used in ordinary carbon paper whereby upon impact of a type bar of a typewriting machine or upon the application of pressure by a stylus or other writing or printing device or apparatus, portions of the protective layer will become temporarily adhesive in nature and stick to a sheet of paper or the like against which it is positioned. The nature of the protective coating used in the present invention, therefore, is preferably such that at the moment of impact or pressure the protective material will have a higher affinity for the backing sheet than it has for the duplicating material within the layer 2. Thus, the portions of the protective layer 4 deposited upon the backing sheet will adhere to the backing sheet when the backing sheet and master sheet are separated and very little, if any, of the duplicating material will be lost.

Specific examples of materials suitable for the protective layer 4 will be set forth hereinbelow. However, in a preliminary way it may be stated that the protective layer preferably comprises a

suitably flexible, resinous material insoluble in the particular solvent to be used in the duplicating process and insoluble in water. For convenience in manufacture the protective material is preferably soluble or dispersible in a solvent or carrier which will not dissolve the duplicating material when the protective coating is applied.

In Fig. 2 there is shown a preferred form of master sheet including a base sheet 1, layer of duplicating material 2 and protective coating 4 as provided in the form shown in Fig. 1. However, this preferred form of master sheet includes an additional layer 3 of a special parting material interposed between the duplicating material 2 and protective coating 4. Illustratively, the parting layer 3 may comprise a micro-thin coating of a wax or wax-like substance which is too soft or fragile to serve as a protective layer. This parting material is applied as a continuous coating over the duplicating material 2 and the protective layer 4 is then applied as a continuous coating over the parting material 3.

The layer 3 of parting material is particularly advantageous when the duplicating material in layer 2 is of a composition having rather great affinity for the resinous protective layer 4. When the duplicating material is high in wax content, its affinity for the protective layer 4 may be so low that the parting layer may be dispensed with if so desired, but when the duplicating material is of an oily or greasy nature for example, the parting layer 3 is desirable in order to avoid or reduce wasteful transfer of duplicating material to the backing sheet along with the protective layer. A preferred material for the parting layer 3 is carnauba wax although other similar natural or synthetic waxes may be used. In general, the material or wax selected should be soluble or dispersible in a solvent or carrier which will not dissolve the duplicating material when the parting layer is applied. Furthermore, the solvent or carrier should have a boiling point such as to permit drying at temperatures below the melting point of the duplicating material. Carbon tetrachloride is the preferred solvent for carnauba wax.

In Fig. 3 there is shown a method of assembling the master sheet of the present invention with a backing sheet 5 upon the platen 6 of a typewriter. The backing sheet 5 is placed in contact with the platen 6 and the master sheet is positioned with the protective coating 4 held against the backing sheet 5. The master sheet may be of either of the forms shown in Figs. 1 and 2 but for the purposes of illustration, the Fig. 2 form has been chosen. The parting layer 3 and layer of duplicating material 2 of the master sheet are shown in proper relationship and the base sheet 1 lies uppermost, the uncoated surface thereof being exposed to type bars 7 of the typewriting machine. It will be understood that the master sheet may be used with or without the usual typewriter ribbon and that if the ribbon is used, a readable copy of the text will be formed on the uncoated or exterior surface of the base sheet 1. Impact or pressure of the type bar will be transmitted through the base sheet and the various layers of the material thereon to transfer local areas of the protective coating 4 and parting layer 3 to the upper surface of the backing sheet 5.

In Figs. 4 and 5 there is shown in diagrammatic and exaggerated form the operation of the master sheet of the present invention. The type bars 7 indent the base sheet 1 as indicated by the depressions 8. Local areas 9 of the protective

layer will be deposited upon the surface of the backing sheet 5. The micro-thin parting layer 3 will be broken in these same local areas and portions 10 thereof will adhere to the portions 9 of the protective layer. When the prepared master sheet is removed from the typewriter and separated from the backing sheet, as shown in Fig. 5, the portions 9 and 10 will remain on the backing sheet and portions 11 of the duplicating material will be exposed in an otherwise continuous coating of protective material 4. These exposed areas will be available for the formation of copies in any of the various manners well-known in the art.

In Fig. 6 there is shown a modified assembly in which a master sheet incorporating the features of the present invention may be used. The master sheet is similar to the ones described in connection with Fig. 1 or 2 and may comprise a base sheet 15 having a continuous coating 16 of duplicating material thereon upon which may be superimposed, if so desired, a continuous micro-thin coating of parting material 17. A layer or coating of protective material 18 is superimposed upon the duplicating material or upon the parting layer if the latter is provided. The master sheet thus formed is superimposed with the coated side down upon a backing sheet 19 beneath which may be positioned any desired number of inter-leaved pencil carbon sheets 20 and writing paper sheets 21. As shown in the drawing, there are two writing sheets and two pencil carbons for the purpose of forming duplicate and triplicate copies of the data written upon the upper surface of the base sheet 15 of the master sheet.

The embodiment shown in Fig. 6 is of unusual value in salesmen's order books or the like. An ordinary pencil may be used for writing upon the upper surface of the base sheet 15. Duplicate and triplicate pencil carbon copies will be made of such material and at the same time the protective coating 18 and parting layer 17 of the master sheet will be locally transferred to the backing sheet 19. When it is desired to form a number of copies of the sales sheet, the master sheet may be removed from the sales book, the backing sheet 19 stripped therefrom and the master sheet will be available for the production of spirit-duplicated copies.

Specific examples will now be given of several master sheets embodying the present invention:

*Example 1.*—A base sheet of paper or other flexible sheet material suitable for use as a master sheet is coated with a suitable duplicating material preferably comprising a mixture of dye and wax, the dye being of a type that is soluble in a duplicating fluid such as an alcohol mixture or other solvent. The coated side of the base sheet is next coated with a carbon tetrachloride solution containing eight per cent by weight cumarone indene resin (for example, resins of the types disclosed in U. S. Patents 1,705,857; 1,770,281; 1,770,283; 1,922,342; 1,990,215; 2,047,246 and 2,092,999) to which is added one per cent by weight a plasticizer such as "Herculyn" made by the Hercules Powder Company. The coating thus applied is dried at a temperature below the melting point of the wax-dye composition in the duplicating layer, the boiling point of carbon tetrachloride being sufficiently low to permit drying at temperatures below the melting point of the various waxes ordinarily used in the wax-dye duplicating layer. The master sheet thus prepared may be used in

either of the manners discussed herein or it may be used in any of the spirit duplicating systems in which master sheets prepared by known processes may be used. The plasticized resin of the protective layer will be found to be stable at room temperature and entirely free from any tendency to smudge or stain surfaces with which it may come into contact. The resinous layer, however, is readily transferable to a backing sheet upon impact or pressure incident to application of printed matter or other indicia to the master sheet for duplication. In this latter connection the resinous protective material is rendered temporarily sticky as a result of the heat produced by such impact or pressure and in this condition is readily adherent to the backing sheet.

*Example 2.*—A master sheet is prepared as in Example 1 except that after the duplicating material has been coated upon the base sheet, a thin film of a one per cent solution of carnauba wax in carbon tetrachloride is applied directly to the exposed surface of the duplicating material. The quantity of carnauba wax thus applied is very small and after drying, there will be left a micro-thin layer or coating which serves as a parting layer as discussed above. The parting layer is dried at a temperature below the melting points of the duplicating material and the carnauba wax. A protective coating comprising any of the resinous materials specified in Example 1 is then placed over the film of carnauba wax and dried as described in Example 1. The micro-thin layer of carnauba wax has very little affinity for the wax-dye composition in the duplicating layer and a greater affinity for the resinous material in the protective layer. The master sheet of the present example may be used in the same manner as that disclosed in Example 1. When the master sheet is written upon, selected areas of the resinous protective layer and the wax parting layer will be deposited upon the backing sheet. When the backing sheet is removed, there will be substantially no duplicating material carried along with the protective layer because of the low affinity between the duplicating material and the carnauba wax.

*Example 3.*—A base sheet is coated with a duplicating material and with a micro-thin layer of carnauba wax as in Example 2. A protective layer is next applied which comprises a carbon tetrachloride solution containing ten per cent by weight a synthetic resin polymerized from resins in the still residue from coke-oven "light oil" (prepared, for example, in accordance with U. S. Patent No. 2,149,577). After drying at a temperature below the melting point of any of the waxes present, the master sheet is finished. The protective layer in this particular example is adhesive under pressure or impact and produces results very similar to those obtained with the master sheet of Example 2.

*Example 4.*—A base sheet having a layer of duplicating material and a parting layer as described in Example 2, has applied over the parting layer a protective layer comprising four parts carbon tetrachloride and one part benzene in which is dissolved eight per cent by weight resins polymerized from "pure still residues" of the coke-oven process (made, for example, in accordance with Patent No. 2,263,224). The protective coating is dried at a temperature below the melting point of any of the waxes present. The protective coating is adhesive under pressure or impact and the master sheet, according to the pres-

ent example, may be used with results substantially identical with those of the master sheet of Example 2.

*Example 5.*—A base sheet having a layer of duplicating material and a parting layer as described in Example 2, has applied over the parting layer a protective layer comprising a solution in carbon tetrachloride of seven per cent by weight resins polymerized from indene and methyl indene (a commercial example is Pecco-Var C-120 made by Pennsylvania Industrial Chemical Corp.). The protective coating is dried at a temperature below the melting point of any of the waxes present. The protective coating is adhesive under pressure or impact and the master sheet, according to the present example, may be used with results substantially identical with those of the master sheet of Example 2.

*Example 6.*—A base sheet having a layer of duplicating material and a parting layer as described in Example 2, has applied over the parting layer a protective layer comprising a solution in carbon tetrachloride of seven per cent by weight a resin polymerized from styrene and its homologues (a commercial example is Piccolastic A-75 made by Pennsylvania Industrial Chemical Corp.). The protective coating is dried at a temperature below the melting point of any of the waxes present. The protective coating is adhesive under pressure or impact and the master sheet, according to the present example, may be used with results substantially identical with those of the master sheet of Example 2.

*Example 7.*—A base sheet having a layer of duplicating material and a parting layer as described in Example 2, has applied over the parting layer a protective layer comprising a carbon tetrachloride solution containing seven per cent by weight resins from the polymerization of beta pinene (a commercial example is Piccolyte S-115 made by Pennsylvania Industrial Chemical Corp.). The protective coating is dried at a temperature below the melting point of any of the waxes present. The protective coating is adhesive under pressure or impact and the master sheet, according to the present example, may be used with results substantially identical with those of the master sheet of Example 2.

The particular resinous coatings set forth in the above specific examples have been selected because they are readily available and have the characteristics essential to the present invention. It will be noted that in most instances no plasticizers are used, the particular resins having sufficient flexibility without such plasticizers. However, it will be appreciated that as in the case of the cumarone indene resins a plasticizer may be used in connection with resins otherwise insufficiently flexible. Thus, many resins not mentioned herein will suggest themselves to those skilled in the art and may be adapted to the present invention by the selection of suitable types and quantities of plasticizing materials.

In order to be suitable for use as a protective coating material in the present invention, a particular material must have the following characteristics all of which are possessed by the illustrative materials set forth in the above specific examples. The material must be capable of being coated as a very thin, continuous film, either as a melt or as a solution or dispersion. The material must be non-tacky at normal office temperatures and should not be soluble in or swelled by any of the solvents normally used as duplicator fluid. Alternatively the material may be

insoluble in one or more specific duplicator fluids and the master sheet may be used only with such fluids. The film of material also must be insoluble in water in order that the moisture normally present on an operator's fingers will not damage the film. The material must be of such nature that the film will become sticky or adhesive to paper or other suitable backing material at the temperature produced by the blow of a typewriter type bar or the pressure of a pencil, stylus or printing press type. In this connection the material will be satisfactory if it has a ring and ball melting point between 70° and 120° C. The film of material in the protective layer must not be brittle at normal office temperatures and therefore, the material selected should have this characteristic or should lend itself to modification by plasticizers to have such characteristic. As pointed out above, certain materials having all of the characteristics herein set forth will have differing affinity for a particular duplicating material and as a matter of fact, different duplicating materials differ quite widely in respect of tackiness and the like. Accordingly, the micro-thin parting layer will be found to be of the greatest value in any combination of duplicating material and protective material between which a relatively great affinity exists. The parting layer has been included in each of Examples 2 through 7 without particular regard to the materials in the duplicating and protective layers. While it is preferred to use the parting layer in each of these examples, it will be realized that the layer may be omitted without rendering the master sheet inoperative. When the parting layer is used very little, if any, of the duplicating material will remain adhered to the backing sheet within the areas of transfer of the protective layer thereto. If the parting layer is omitted, varying quantities of duplicating material may be lost in this manner depending upon the affinity between the particular duplicating material and the particular protective material selected. Thus, in certain instances the number of copies available from a prepared master sheet may be reduced by varying amounts in the event the parting layer is omitted. Therefore, since the parting layer may be rapidly and inexpensively applied in the manufacture of the master sheet blanks, the ability to obtain even a few additional copies may well offset the slight additional cost incurred when the parting layer is included. From the above detailed description and specific examples it will be apparent that the master sheet of the present invention accomplishes the objects set forth hereinabove.

We claim:

1. A method of duplicating which comprises providing a master sheet having a layer of duplicating material soluble in a duplicating fluid, a layer of protective material insoluble in said duplicating fluid overlying said layer of duplicating material, and a micro-thin parting layer of wax interposed between said layer of duplicating material and said protective layer; transferring localized areas of the protective layer and parting layer of said master sheet to a backing sheet by the application of impact or pressure; separating said backing sheet and said master sheet to expose the duplicating material in said master sheet only within said localized areas; and forming a plurality of duplicate copies from the duplicating material thus exposed.

2. A method for forming a plurality of copies of desired indicia comprising providing a master

sheet having a continuous layer of duplicating material on one face thereof, said duplicating material being soluble in a duplicating fluid, a continuous layer of protective material overlying said duplicating material, and a continuous micro-thin parting layer of wax interposed between said layer of duplicating material and said layer of protective material, said protective material and said parting layer material being impact or pressure-transferable and said parting layer material being readily separable from said duplicating material; assembling said master sheet with a backing sheet, the protective layer of said master sheet being in face-to-face relation with a surface of said backing sheet; transferring portions of said protective layer and said parting layer to said backing sheet in the form of the indicia desired to be duplicated; separating said backing sheet and said master sheet to expose the duplicating material of said master sheet within the areas defined by said indicia; and forming a plurality of duplicate copies of said indicia by bringing the surface of said master sheet having said protective coating thereon into contact successively with a plurality of copy sheets in the presence of 25 duplicating fluid.

RAY BENNETT KELLER.  
HARROLD BOWMAN DAWSON.

## REFERENCES CITED

The following references are of record in the file of this patent:

## UNITED STATES PATENTS

| Number       | Name      | Date          |
|--------------|-----------|---------------|
| 894,815      | Clarke    | Aug. 4, 1908  |
| 1,845,568    | Strawn    | Feb. 16, 1932 |
| 1,864,097    | Sherman   | June 21, 1932 |
| 10 1,925,235 | Dixon     | Sept. 5, 1933 |
| 2,086,011    | Whitmore  | July 6, 1937  |
| 15 2,163,958 | Neidich   | June 27, 1939 |
| 2,181,864    | Bjorksten | Dec. 5, 1939  |
| 2,188,590    | Bjorksten | Jan. 30, 1940 |
| 2,398,779    | Dalton    | Apr. 23, 1946 |

## OTHER REFERENCES

Printing Inks by Ellis; Reinbold Pub. Corp., New York, N. Y. (1940); pages 314-320. Copy in 20 Div. 17.